

## UNITED STATES PATENT OFFICE

WILLIS A. BOUGHTON, OF CAMBRIDGE, MASSACHUSETTS, ASSIGNOR TO BENNETT BOX CO., OF BOSTON, MASSACHUSETTS, A CORPORATION OF MASSACHUSETTS

## ART OF STIFFENING

No Drawing.

Application filed December 15, 1922. Serial No. 607,218. 117-157

This invention relates to improvements in the art of stiffening. More especially it relates to improvements in processes by which sheet materials of industrial utility, such as cloth, leather or paper may be made stiffer than they are by nature. It is especially useful for various articles of manufacture such as hat shapes, counters of shoes, and kindred fabrications, including box toes of shoes. 10 It belongs to the general class in which material is applied in liquid form at ordinary temperatures, and the stiffening results from atmospheric drying.

In the manufacture of toe boxes, for which the invention has important utility, it is particularly desirable to provide so that the box can be bent in by pressure but will immediately resume its original form when the pressure is removed. It is one object of the invention 20 to provide such a box.

The invention also combines certain advantageous industrial characteristics which have long been sought in the general art to which the invention relates. Among these are that the materials employed should be inherently 25 inexpensive, and should be easily obtainable in abundant quantities and standard quality. Another is, that the result of the treatment should be permanent, the material maintaining whatever degree of stiffness it acquires, or 30 imparts, without being easily affected by moisture, as are glues; nor by heat, as are waxes, asphalts, pitches and shellacs. Others are that it should be non-putrescible; should 35 be odorless, and remain so when heated or wetted; should not injuriously affect the sheet 40 materials with which it is used, nor alter their properties within a reasonable length of time, nor deface them, as when a black or colored waxy or pitchy stiffener sometimes permeates 45 to and discolors the face of a white shoe leather. It should be safe when handled and stored in quantities in the factory; and should not entail the storage or handling of any dangerous substance for the working of it, as does 50 celluloid, for example. It should moreover be easy to handle in the factory; and should produce the desired stiffness with sufficient rapidity. Furthermore it is desirable to be able to predetermine the degree of stiffness.

which the box shall have, because sometimes a marked degree of flexibility is desired and for other purposes a practically unyielding box is desired. The present invention attains all of these standards, and in so doing combines in itself characteristic advantages that have never heretofore, so far as I am aware, been associated in any practicable stiffening process or stiffened product. 55

In the best form in which I at present contemplate using it these objects are attained by applying a substance which is made liquid by the presence of water, but which is capable of conversion to solid form while still containing a very considerable amount of water. 60 The stiffening is accomplished by solidification in the presence of considerable moisture. I have found suitable material for this in the high ratio silicates of alkali metals, that is, silicates containing the higher proportions 70 of silica to soda or potash. Such may become "dry" and hard, that is, may acquire the aspect and physical effect of substances that are free from moisture, and yet may at the same time contain as much as 50 per cent of 75 water. Under these circumstances, if a proper concentration of the liquid silicate be used, as for example one containing less than 60 per cent of water, the difference between its fluid state, in which it can be conveniently 80 applied to and can penetrate a supporting medium such as felt or paper, and its solid state in which it makes that medium stiff, means that the "drying" is accomplished by removal of only small percentage of its water content. 85 With other water-soluble stiffening materials, e. g. glues, the difference between water content in liquid state and water content in solid state is usually much more than this. For the purposes of the invention sodium silicates having a formula of the order of  $\text{Na}_2\text{O}(\text{SiO}_2)_x$  or  $\text{Na}_2\text{O}(\text{SiO}_2)_y$  seem to have the molecules in 90 micelles or other arrangement of such size and character that a certain residual quantity of the water is associated with the molecules of the solids far more intimately than ordinary water of solution. When a film of such sodium silicate is exposed to evaporative influence, the material at the surface of the film 95 quickly reduced to a semi-solid, non-sticky 100

state, in which the material bearing it may be handled conveniently, and from which state its drying continues till the whole becomes a hard, horny mass. I have found these effects present in the said silicates having high ratio of silica to sodium, much more satisfactory than in sodium silicates of lower silica to sodium ratio. The high ratio silicate gives a greater stiffness and strength of film when compared with the equal ratio sodium silicate having the same amount of anhydrous material. The ratio of silica to alkali does not affect the amount of total solids present in any case, but merely the proportion of the two radicals composing any weight of anhydrous material; thus, if there be 40 per cent of anhydrous material present in the two varieties, the  $Na_2O$  and the  $SiO_2$ , may in the latter be in equal molecular proportions, and in the former may exist in the ratio of 1 to 4. The water present is variable in amount. It will be understood that the formulas herein given are merely illustrative and do not necessarily convey the exact idea of the way in which the alkali and silica radicals are grouped, or may be supposed to be grouped.

Moreover, although the high ratio silicate solution feels alkaline, it does not act chemically alkaline as do the low ratio sodium silicates. It does not rot cloth and when once dried is less soluble in water and less subject to deterioration. It will be understood that the word "soluble" is used herein in its popular sense of becoming liquefied on addition of water, without touching the technical question whether a "soluble silicate" goes actually into true solution or into suspension, or otherwise. In the high ratio sodium silicate micelle or molecule-grouping, the alkali is less firmly attached to the grouping than is the sodium in such a salt as sodium chloride. The approximate balancing of its attachment, or balancing of alkalinity, is a matter of great advantage in the present invention, as compared with other stiffeners such as glue.

It is sometimes desired to apply a stiffening agent to a sheet with the aid of an auxiliary sheet as a supporting medium. The sodium silicate solution combines particularly well with paper felt, untreated roofing felt, blotting felt, and unsized paper matte, bleached or unbleached cotton or woolen felt, or felted or flannelled surfaces, or even surfaces without nap, as, for example, in the manufacture of a box toe. It is recognized as a technically difficult process to saturate thoroughly sheet materials such as those named with a stiffener such as glue; but the silicate solution of the invention readily soaks into such fibers and fills the pores. It is my belief that this action is due to the fact that radicals of the sodium silicate molecule, in whatever form it exists in these high ratio silicates, associate sufficiently when the chemical co-

tions call for dissociation, to yield a small proportion of free hydroxyl ions; that there is usually more or less grease present on felt of any kind, or cloth, and that the hydroxyl ions which attend the silicate solution are efficient in de-greasing the fiber so that the solution readily enters and may effect both inter-fibrous and intra-fibrous penetration.

As with other stiffeners, e. g. casein or glue, a silicate stiffening will absorb a certain amount of water when exposed to water vapor or liquid; and it is therefore ordinarily desirable to protect such stiffeners from the action of water. One of the ways in which this may be done is by laying on a coat of waterproofing material, of which suitable types are already in common use. Such a protective coating should form a continuous film. To this end it may either be applied in a thick and hot condition, so that when cooled it is approximately solid; or it may be applied as a thin sheet supported on an auxiliary light thin medium such as tissue or other paper. When the waterproofing treatment is applied to a sheet of material which is later to be softened as, for example, for the lasting of a box toe, it is particularly desirable that the waterproofing should be only on the surface, as distinguished from coating each fiber, so as not to prevent the stiffener from taking up enough water to become sufficiently soft to allow of easy lasting of the box toe.

The contradictory requirements that the stiffening material should be waterproof and yet should be capable of taking up water so as to become soft for the lasting may also become harmonized, according to the invention, by using an auxiliary waterproof layer of material sewed or otherwise permanently attached to the underside of the box, which may have been prepared as by skiving. For example, a well known waterproofing material consists of thin strong paper coated with a continuous waterproofing layer which holds on it a strengthening sheet of coarse mesh cloth. The attachment of this material to either side of the skived box allows the box to be softened by the action of water on both sides, for the sewed-on material can be held away during dipping, or, if not so, the water can enter at the edges; and yet, when the box has been lasted in the shoe, this material affords a water-proof layer which satisfactorily prevents access through the sheet material of moisture from without, or from perspiration, that might soften the box. Boxes may be built up in any other suitable way, as for example from two or more layers of paper or cloth, to which the silicate solution, acting as adhesive, may attach one side of the water-proof material above described. The whole sheet thus integrated may then be allowed to dry, with or without pressure, and then be cut to shape, skived if

desired, and wetted before lasting, long enough for water to penetrate the un-waterproofed side sufficiently to allow of easy lasting. In this case sewing is not necessary as the stiffening material holds the waterproofing material.

The stiffener may however be waterproofed when there is no such sheet protection. I do this by rendering the surface of the silicate layer in the integrated sheet or stiffened box insoluble, thereby protecting the body of silicate within the stiffened sheet of cloth, paper or felt from attack by the moisture which would soften it if it had access thereto. Such a stiff supporting sheet of felt, etc., can be waterproofed chemically with respect to one or both surfaces, after the sheet has been saturated with silicate and allowed to dry. One method of doing so consists in spraying or painting the surface thereof with an acid solution, or with the solution of a substance which contains free hydrogen ions, or collodion or other substance which will precipitate gelled silica from soluble silicates. By this means a layer of insoluble silica is precipitated on the surface as a body whose physical form is rather similar to that of the sodium silicate solution, in that it is a colloid and occupies considerable volume for the mass of anhydrous material present, but which is not easily soluble in water and which as a film is more continuous because of its colloidal quality than a film made of an ordinary precipitated salt; and which, probably because of its colloidal quality and the difficulty with which one colloid passes through another, appears to have a marked and positive effect in preventing the soluble sodium silicate within the said felt or other sheet from dissolving out of it, although at the same time it does not markedly hinder the softening of the sodium silicate within. The depth of the layer of insoluble silica thus formed on the surface of the felt or other medium depends upon the strength of the acid and the length of time of application. Moreover, because the film deposit is a colloid or of a gelatinous nature and occupies considerable volume for the mass of anhydrous material present, there is no marked change in volume, no shrinking or swelling with incidental wrinkles or cracks, resulting from the treatment.

An insoluble coating for the felt or other material containing the silica solution may also be provided by precipitating an insoluble silicate on the surface by treatment with a solution of a soluble salt which contains an ion of a metal forming an insoluble silicate. Almost any soluble metal salt except those of the alkalies, can be used for this purpose, such as calcium, zinc, magnesium, aluminum, etc.

The solution for treating the surface may be applied when the sodium silicate is in a moist, partly dry, or air dry condition. This,

industrially, gives a great range of freedom as to the time for applying the treatment. It allows material to be prepared, dried, kept dry in storage, and ultimately to be used with or without the waterproofed surface as may be desired. The degree of concentration of the acid employed may vary, depending on the dryness of the sodium silicate, so as to avoid adding unnecessary water. If the stiffener be still wet the acid may be far more concentrated.

It is another feature of the invention that the qualities of stiffness and flexibility of a stiffened box may be varied in degree, and the brittleness decreased. A supporting medium such as felt, or felted cloth or paper, or cloth sheet, is relatively hard when heavily impregnated with a silicate solution and dried. If it be desired to have a shoe box that is somewhat more flexible, almost any desired degree of flexibility may be obtained by the addition of the requisite amount of glycerine, soap or soap solution (particularly so-called soft soap) a drying or non drying oil, such as cottonseed oil or linseed oil, which can be emulsified with the silicate solution, or any desired combination of these softeners. This may be added to the silicate solution and thoroughly incorporated with that solution, before impregnating the fibers of the said supporting medium.

By the use of a fatty oil, as above mentioned, advantages of particular importance may be attained. I have discovered that oils of vegetable or animal origin, such as cottonseed and linseed oil will emulsify easily, rapidly and completely with silicate solution so as to form a mixture which can be applied in every way like the silicate solution and will dry at approximately the same speed or somewhat more slowly. The oils appear to be carried in an extremely finely divided state everywhere that the silicate penetrates and they result in the lubrication of the air dried micelles to such an extent as to produce a springy flexible sheet. A non drying oil, such as cotton seed oil, keeps its oily properties and maintains the flexibility. A drying oil in the emulsion produces a stiff sheet which takes on the qualities of both silicate stiffness and varnish toughness. In this respect the integrated sheets attain to a marked degree that quality of springiness which is much desired for the so-called flexible box toe, and have a comparatively high bending coefficient. That is, they can be bent into a curve which, if a section of a circle, may be of pretty small radius, and may form a complete circumference, yet when the pressure is released they immediately resume practically the original flatness; and in general, when bent they snap back with somewhat the effect of a sheet of tempered steel, or of celluloid.

An advantage of the use of oil emulsion is

that the layer of oil around and in the silicate acts markedly as a waterproofing agent. The oil passes liquid water easily to the silicate and so, in the case of a toe box, does not interfere with the softening by liquid for lasting; but such a sheet is less affected by water vapor than are the non-emulsion silicates. This is a feature of importance where it is desired that a box withstand the moisture 10 from perspiration, without having a homogeneous waterproofing layer. By including glycerine and oil in the emulsion a waterproofed sheet may be made of superior resilience, due to the glycerine.

15 Without employing the foregoing, a somewhat similar effect can be produced by selecting and using for the active stiffening agent a silicate solution containing a smaller proportion of silica to sodium, in which the formation of hydroxyl ions by dissociation gives, in effect, a solution of sodium hydroxide with the sodium ions of the silicate molecules. Caustic alkalies such as sodium hydroxide, being markedly deliquescent, will keep the 20 silicate film from drying to so great a degree. For example, experiment showed that a 1 to 1 ratio solution did not become even surface dry in twenty-four hours. Hence by proper proportioning, almost any desired degree of 25 softness may be attained for a stiffener of material. A similar effect may be produced by the addition of any other soluble deliquescent salt which does not react chemically with sodium silicate; or, without such 30 addition, by reducing the residual amount of dry stiffening material, as by squeezing out a part immediately after application or by applying it in more dilute form, thus in either case making less dry material in a given 35 volume.

The stiffened product thus far described is inorganic, so far as the stiffening material is concerned, and therefore will not decay or mold. When sufficiently air dried it is 40 not softened by the action of heat under temperatures at which leather itself is injured. The materials required are low in cost and easily available in large quantities in the market. The material is easy to handle in 45 the factory. Being applied in liquid form without heat it can be applied with great speed. As it becomes soft by mere addition of water, and without heat, there is neither danger nor expense for heating. As it dries 50 with comparative rapidity, space required for handling a large quantity of stiffened sheet material, or articles such as shoes or hats in which it is embodied, is small.

Having thus described the general nature 55 of the invention, an illustrative example of the manner of practicing the same will be given.

The material preferred for the active agent of the stiffener is sodium silicate having a relatively high ratio of silica to sodium, as

illustrated by the hypothetical formula  $\text{Na}_2\text{O}(\text{SiO}_4)$ . This may be prepared by a known process. It may be applied by any suitable method of spreading and impregnation. For example, a sheet of material such as felt, cloth or paper, may be run over a roller whose under portion is immersed in a bath of the liquid sodium silicate. The liquid is brought up from the bath by the rotating roller as the sheet of felt is drawn over the roller. The liquid which is thus drawn up soaks into the felt. As the latter moves away, the surface of the sodium silicate which it has acquired loses water by evaporation and quickly becomes non-adhesive, which makes the coated sheet more easy to handle. Care should be taken that the skin of solidified particles resulting from the evaporation is sufficiently formed before two treated layers of the sheet are placed in contact with each other for storage else they will adhere together.

Where deep penetration of the sheet by the stiffener is not desired, the liquid stiffening material may be sprayed upon the surface 90 of the sheet, either or both the sheet or the sprayer being in motion, the one relative to the other. Any suitable spraying apparatus may be used for this purpose, as for example such as works by a jet of compressed air, commonly called an atomizer, or one in which the fine subdivision of the liquid results from other characteristics of the jetting apparatus. In either case care should be taken that the superficial solidification of particles, due to evaporation of moisture which begins immediately upon issue of the finely sub-divided liquid particles from the nozzle, shall not proceed too far before they become settled on the material, for in that case the film on the sheet 100 material will not have that continuous character which is desired, and which is attained, according to the invention, by laying on the sheet a liquid film of the drying material and then drying that film so as to remove a part 105 of its associated water without destroying its film characteristic. I have found the higher ratio silicates, and especially those having the ratio of 3 to 1, or of 4 to 1, to give greater strength of film than solutions of lower ratio silicates wherein there is present the same amount of anhydrous material and the same percentage of water. In the case of an easy flowing solution of high ratio silicate which I have used, the original water content of the 110 commercial product purchased for use in the process may be reduced markedly by evaporation, leaving a product which in that case contains approximately 42 per cent of water and which nevertheless is solid and free from 115 apparent moisture; and the drying occurs with sufficient rapidity to make the material and method of treatment commercially valuable for stiffening the articles to which it is applied. If quicker solidification after ap- 120 125 130

plication is desired, more concentrated silicate solution may be applied. I believe the rapidity of drying to be due in part to the fact that in these high ratio silicates the molecules are organized in large hydrated units of colloidal nature in which a considerable portion of the water is held fast, and only a portion is free to evaporate at ordinary temperatures; and that the extending of this liquid in a film, or in globules when applied by spraying, produces such a large area of evaporative surface that whatever small part of water is free departs with great ease, quickly forming the hard skin which, as evaporation proceeds, rapidly extends from the surface into and completely through the sheet or layer of stiffening material.

I have found that a satisfactory light weight box toe can be made by laying the above-described stiffening material directly on the undersurface of the leather cap and then proceeding through the lasting process as usual. If the leather has been thus previously impregnated and allowed to dry it may be dipped in or painted with water or a suitable softening solution, on the under side with water just prior to the lasting. If not thus prepared it may be painted or sprayed, just prior to lasting, with the stiffening material in such concentration or such viscosity that it will stay on the surface rather than penetrate the fibers of the leather, and the lasting is then carried out as usual, producing a light but firm toe.

Where the stiffener is to be protected from water during subsequent use, it may be desirable to lay a waterproof layer against the leather before treating with the stiffening material, or to provide waterproofing otherwise, as above described. Where it is desired to combine in a toe the qualities of strength and light weight, this can be done and predetermined at will, according to the needs of the case because a wide latitude is afforded, when the stiffener of the invention is used, for choosing a suitable number and variety of layers in the composite box; or choosing or varying the thickness of the supporting medium, such as cloth, paper or felt (which latter especially may act as a carrier for a greater or less thickness of the stiffener according to the greater or less thickness of the felt); or for applying the stiffener to the under surface of the toe cap; or varying the concentration or amount of stiffener used in the box.

Where it is desired to hasten the drying of a silicate stiffener of the type hereinbefore described the stiffening may be accelerated, so as to be quickly completed either temporarily or permanently, so that in the case of a shoe with box toe the last can be pulled within a few minutes after being lasted. These two methods are as follows:

The temporary stiffening, which permits

the last pulling, is effected by dusting on the surface of the moistened and completely flexible box, just before lasting, a powdered salt which will take up water to form a crystal layer. The salt should be harmless and inexpensive and should in no stage of its application or use interfere with other processes or the satisfactory use of the shoe. Such salts are, particularly, sodium-sulphate and sodium-carbonate, both in the anhydrous condition. These salts in the presence of the right amount of water will take up water and become crystalline; and in the process of rapid stiffening of the silicate box these crystals form a comparatively hard layer over the surface of the box, which allows the last to be withdrawn promptly. Within a half an hour or an hour however, the additional water in the silicate box will soften this crystal layer again, so that the hardening effect is merely temporary; but by that time evaporation will have proceeded to such a point that the toe holds its shape. The temporary stiffening in this case is due to two actions: First the anhydrous salt withdraws some water from the silicate, rendering it stiffer through that withdrawal of water; and, second, the anhydrous salt itself forms a stiffening layer through its crystallization.

The acceleration to a permanent stiffening may be effected by similarly dusting, on the surface of the moistened and flexible box, a white insoluble oxide of an element that forms an insoluble silicate. Such oxides are magnesium oxide, zinc oxide, aluminum oxide and calcium oxide; the last is less desirable because of its recognized caustic qualities. In the case of these oxides reaction takes place between the oxide and the silicate solution to form a dense, hard layer of insoluble silicate. This layer is permanent. It is important that the solidification of this layer be allowed to take place as much as possible free from disturbances, as otherwise the homogeneity of the layer is destroyed.

These materials to produce rapid stiffening may be used with any of the ordinary stiffening formulas elsewhere mentioned herein.

An illustrative example of the practice of the invention would be as follows, illustrating a preferred procedure for application of the invention for certain purposes. Take as ingredients:

Solution of high-ratio silicate-to-soda alkali silicate solution, containing 40% of anhydrous matter, 200 parts, by weight;

Unboiled linseed oil, 7 parts, (boiled oil or varnish may be used);

Glycerine, 9 parts.

If the particular qualities desired in the final product require it, the unboiled linseed oil, boiled oil or varnish, may in part be replaced by a semi-drying or non-drying fatty oil. This and the glycerine have each the property of producing a degree of flexibility.

in the silicate stiffened material; but when the oil is used a degree of water proofing is attained which is absent when glycerine alone is used.

5. An emulsion of these is applied to cloth sheeting, on one or more layers to the extent of from 300 to 1200 grams of mixed solution per square yard. The sheet is then air dried, and may later be dried with heat from steam.

10. When applied to sheet having a nap it may advantageously be applied on the nap side. In a typical case the material may be applied to one side of a sheet; then covered by a second sheet, and then, by application of pres-

15. sure, made to penetrate the second sheet as well as the first. If the material is to be waterproofed by forming a layer of silica gel, the acid may be applied to one of the pieces of cloth by spraying it thereon. The emul-  
0 sion having been worked into the body of the cloth the acid finds it there, and by reaction the acid entirely disappears, leaving the silica as one of the products of the chemical reaction that occurs in the body of the cloth. How-

25. ever, in a preferred arrangement, there is enough of silicate emulsion or solution to soak completely through both pieces of cloth to which it is applied; and in that case the acid when applied immediately meets the

30. silicate and makes its deposit of silica on the outer surface of the composite sheet. For such an acid application of a solution of acetic acid preferably not stronger than 5 or 10% may be used. If waterproofing is to be ac-

35. complished by covering with a layer of waterproofing material, asphalt may be used, for which purpose the asphalt may be made of such temperature and viscosity that when laid on the surface it will form a layer and

40. will not penetrate. The same general principle would cover the use of other waterproofing materials.

It is intended that the patent shall cover, by suitable expression in the appended claims, 45. whatever features of patentable novelty exist in the invention disclosed.

I claim as my invention:

1. A stiffened sheet of material which is 50. flexible by nature and has disseminated through it a solidified soluble silicate and glycerin.

2. A stiffened sheet of material which is 55. flexible by nature, said sheet being rendered stiffer by having associated with it a dried emulsion of a silicate of an alkali metal with a fatty oil.

3. A stiffened sheet of material which is 60. flexible by nature, said sheet being rendered stiffer by having associated with it a dried emulsion of a silicate of an alkali metal with a drying oil.

4. A stiffened sheet of material which is 65. flexible by nature, said sheet being rendered stiffer by having associated with it a dried emulsion of a silicate of an alkali metal with

a mixture of a drying and a non-drying fatty oil.

5. A manufactured shape, such as a toe box, 70. made of sheet material which is flexible by nature and is rendered stiffer by having as-  
sociated with it a dried emulsion of a silicate of an alkali metal wherein the ratio of num-  
ber of silica radicals to the number of alkali oxide radicals is three or more to one, and  
the oil is a drying oil.

6. A manufactured shape, such as a toe 75. box, made of sheet material which is flexible by nature, rendered stiffer by impregnation with an emulsion of a silicate of an alkali metal and oil.

7. A stiffened sheet of material which is 80. flexible by nature, said sheet being rendered stiffer by having associated with it a dried emulsion of a silicate of an alkali metal with glycerine and a drying oil.

Signed at Boston, Massachusetts, this eleventh day of December, 1922.

WILLIS A. BOUGHTON.